

## UNITED STATES PATENT OFFICE

1,995,862

## POLISHING COMPOSITION

Herbert Spencer Polin, New York, N. Y., assignor  
to Polin, Inc., New York, N. Y., a corporation of  
Delaware

No Drawing. Application November 18, 1932,  
Serial No. 643,289

14 Claims. (Cl. 134—24)

This invention relates to a polishing composition and includes both the new composition and the method of making it. The polishing composition contains both wax and soap and combines the functions of a cleaning agent and wax surfacer.

Wax in small amounts may have been added to cleaning compositions, but so far as I am aware there is no soap compound on the market which

10 contains sufficient undissolved wax to form a product which polishes as it cleans. Conversely, soap has been added to wax previously, but never in such an amount that the mixture could be used for cleaning. In my composition, both soap and 15 wax are present in such an amount that each maintains its functional identity. The soap acts as a cleaning agent; the wax acts as a surfacer and preservative. Products which contain a 20 solution of wax in a low boiling organic solvent such as gasoline are not suitable because each fresh application of such a solution dissolves wax already applied to the surface treated. In my product the soap and wax are present as an emulsion.

25 Emulsions containing too little wax fail to deposit an effective wax covering. I find that a mixture containing 10% of wax and ninety percent of soap, oils, etc. is satisfactory for the production of a light wax surfacing and somewhat 30 less wax, for example, 5% may be used, but I prefer to use fifteen percent of wax, and even up to thirty-five percent. With a compound containing more wax than this, I found that during a single treatment, a fresh application of the 35 compound picked up wax previously deposited during the same treatment. An emulsion containing 10 to 35% of wax and a considerable quantity of soap cleans as a soap and has the added property of surfacing with wax. This 40 composition when applied directly to a dirty floor, piece of furniture or automobile, etc. in one rubbing operation effectively cleans the surface, deposits a coating of wax and burnishes it. It 45 is not necessary to clean the surface before polishing it and the composition contains wax in the proper amount for speedy burnishing and effective coverage.

The soap used in the polishing composition 50 may be a household cleaning soap, the base of which is ordinarily a combination of tallow and olive or pine oil saponified with a sodium base. I use twenty or more parts of such a soap in dry powdered form, or I may employ a water solution 55 of such a soap. I compound wax, oil and water

and preferably also casein with the soap in preparing my polishing composition.

I use wax which is not soluble in water. I prefer a wax having a relatively high melting point, that is, a wax which after application will not be affected by ordinary atmospheric temperature changes nor by the friction of contact. Various waxes with a melting point above 75° C. have been used.

5 In order to produce a smooth homogeneous 10 product, I add an appreciable amount of casein or other homogenizer. From about one to ten percent of casein produces a homogeneous, smooth-flowing liquid, and the preparation is lighter in color, than otherwise. Without any 15 casein, or with less than one percent the compound is darker in color and coarser in texture being somewhat granular, with a slight tendency for the sperm oil to separate out. Using more than ten percent of casein, the product tends 20 to become abrasive. Other homogenizers such as albumenose or albumen products and casein derivatives may be used instead of casein. When casein is used, it may be advantageous to add a 25 small amount of any usual casein preservative. A slight alkalinity of the composition will usually suffice.

In preparing the polishing composition, I dissolve the soap in sufficient water to make about 30 fifty percent soap solution and to this I add a non-drying animal or vegetable oil, such as sperm oil. Other oils such as pine oil may be used, although sperm oil appears most satisfactory. Sperm oil by itself is a good cleaning agent. It 35 leaves a dry finish and is very satisfactory for removing grease. I heat the wax with rosin oil and stir the casein into the mixture of the two. I then combine the soap mixture with the wax mixture and thoroughly agitate the two adding more oil if desired to reduce the viscosity of the 40 product. For example, I add fifteen parts by weight of water and eight parts of sperm oil, to thirty parts of an ordinary soap powder which may, for example, have about the following composition:

|                         | Pounds |
|-------------------------|--------|
| Tallow                  | 117    |
| Cocoanut oil            | 40     |
| Caustic soda (35.5° Bé) | 117    |
| Sodium silicate         | 195    |
| Pearl ash lye           | 31     |

I have used other well-known commercial soap compositions with satisfactory results. In a separate vessel, I heat thirty-five parts by weight of 55

a synthetic wax consisting of chlorinated naphthalene wax and eight parts by weight of rosin oil. The wax and rosin oil are heated to the point of bubbling and then I add four parts by weight of casein and thoroughly stir the mixture. The soap and sperm oil solution is well heated and agitated and the wax and rosin oil mixture is stirred into it. I prefer a liquid product and more sperm oil may be added to reduce the viscosity of the resulting product in the event that it will not flow upon cooling. The mixture is then allowed to cool while it is being agitated and is then bottled immediately. The preferred form of the product is a light colored homogeneous liquid polish which may be applied without additional water to the surface to be polished.

Instead of synthetic wax I may use other waxes such as candelilla, ceresine, raphia, etc. Thirty-five parts by weight of any of these waxes may be substituted for the synthetic wax mentioned in the formula.

I am not entirely satisfied with my own explanation of the finishing and polishing action of this compound. The finished product is a rather heavy viscous liquid in a finely divided globular state, each small bubble of which carries a centrally located bit of wax. The detergent action of soap is due to its ability as a colloid to produce deflocculation. Dr. Jerome Alexander in his recent book "Colloid Chemistry" in Chapter X on page 127, stating the latest theory of the action of soap says: " \* \* \* that soap makes dirt particles less adherent to the fabric or surface and to each other". Applying Dr. Alexander's suggestions to my formula, I believe that the action of applying the colloid to a surface forces an exchange between the relatively heavy wax in suspension and the relatively light sediment on the surface to be cleaned, under the agitation of a brisk application with cloth or mop. Since the wax which I employ is not water soluble, its surface adhesion when applied under pressure repels the efforts of the colloid to recover it and continued friction of the applying cloth spreads and burnishes the deposited wax. Since the soap surrounds the wax, it completes its cleaning prior to the depositing of the wax.

I claim:

1. The method of preparing a cleaning and polishing composition which comprises emulsifying water insoluble wax and rosin oil with a solution of soap and an animal or vegetable oil.

2. The method of preparing a cleaning and polishing composition which comprises emulsifying water insoluble wax and rosin oil with a solution of soap and an animal or vegetable oil in the presence of an homogenizing agent.

3. The method of preparing a cleaning and polishing composition which comprises adding a heated aqueous solution of soap and animal or vegetable oil to a heated mixture of water-insoluble wax, rosin oil and casein and emulsifying.

4. The method of making a cleaning and polishing composition which comprises heating a

fifty percent solution of water and soap to which sperm oil is added and then adding this to a heated mixture of water-insoluble wax and rosin oil and emulsifying in the presence of an homogenizing agent.

5. The method of making a cleaning and polishing composition which comprises heating a fifty percent solution of water and soap to which sperm oil is added, adding this to a heated mixture of water-insoluble wax and rosin oil containing casein, the amount of wax being at least twenty percent by weight of the whole, and emulsifying.

6. A cleaning and polishing composition which is an emulsion containing a small amount of water, sperm oil, at least ten percent of high melting point wax and at least twenty percent of soap.

7. The method of preparing a cleaning and polishing composition which comprises emulsifying water insoluble wax and rosin oil with a solution of soap and an animal or vegetable oil, the composition to contain 10 to 35% of wax.

8. The method of preparing a cleaning and polishing composition which comprises emulsifying water insoluble wax and rosin oil with a solution of soap and an animal or vegetable oil, the composition to contain 10 to 35% of wax and at least 20% of soap.

9. The method of preparing a cleaning and polishing composition which comprises emulsifying water insoluble wax and rosin oil with a solution of soap and an animal or vegetable oil in the presence of an homogenizing agent, the composition to contain 10 to 35% of wax.

10. The method of preparing a cleaning and polishing composition which comprises emulsifying water insoluble wax and rosin oil with a solution of soap and an animal or vegetable oil in the presence of casein, the composition to contain 10 to 35% of wax.

11. The method of preparing a cleaning and polishing composition which comprises emulsifying water insoluble wax and rosin oil with a solution of soap and an animal or vegetable oil in the presence of an homogenizing agent, the composition to contain 10 to 35% of wax and at least 20% of soap.

12. The method of preparing a cleaning and polishing composition which comprises emulsifying water insoluble wax and rosin oil with a solution of soap and an animal or vegetable oil in the presence of casein, the composition to contain 10 to 35% of wax and at least 20% of soap.

13. A cleaning and polishing composition consisting of an emulsion containing 10 to 35% of water-insoluble wax having a high melting point, at least 20% of soap, oil and water.

14. A cleaning and polishing composition consisting of an emulsion containing 10 to 35% of water-insoluble wax having a high melting point, sperm oil, rosin oil, and 40 to 70% of a fifty percent solution of soap.

HERBERT SPENCER POLIN.